

J. L. HERMAN.

PROCESS OF COATING AND TREATING MATERIALS HAVING AN IRON BASE.  
APPLICATION FILED MAR. 6, 1922.

1,430,649.

Patented Oct. 3, 1922.



By

Inventor

Joseph L. Herman  
Chas. Abbott

Attorney

Patented Oct. 3, 1922.

1,430,649

# UNITED STATES PATENT OFFICE.

JOSEPH L. HERMAN, OF PEORIA, ILLINOIS.

## PROCESS OF COATING AND TREATING MATERIALS HAVING AN IRON BASE.

Application filed March 6, 1922. Serial No. 541,561.

To all whom it may concern:

Be it known that I, JOSEPH L. HERMAN, a citizen of the United States, a resident of Peoria, in the county of Peoria and State 5 of Illinois, have invented new and useful Improvements in Processes of Coating and Treating Materials Having an Iron Base, of which the following is a specification.

This invention has reference to a process 10 of coating and treating materials having an iron base and particularly the coating and treatment of wire used in the fence industry and for telephone and other purposes.

The principal object of the invention is to 15 subject the coated material to a simultaneous heat-treatment and annealing during the continuous process of coating such material and preferably immediately upon the material leaving the molten coating bath in 20 which the material is immersed or through which the material is moving. Such heat-treatment has for its object an improved coating which will be more resistant to atmospheric rusting and corroding conditions 25 than is ordinary galvanized wire, and which further will permit a heavier coated wire to be used in wire fabricating machines without causing the coating to crack or flake off, as is the case with heavily coated gal- 30 vanized wire coated by ordinary processes; the annealing of the material being for the usual softening purposes.

The invention has for a further object to 35 subject the coated material to a heat-treatment or to a simultaneous heat-treatment and annealing in an air or oxygen free atmosphere.

The invention has for a further object to 40 apply a heavier coating on the wire with a shorter immersion in molten zinc than is the case with ordinary galvanized wire carrying the heavier coating.

A further object of the invention is to 45 permit the use of higher speeds for galvanizing wire than can be used under the ordinary galvanizing process where heavier coatings are desired and at the same time causing a heavier coating to be formed on the wire.

50 This application is a companion to the application for patent filed by me on February 10, 1922, bearing Serial Number 535,660 for a process of coating and treating materials having an iron base. The invention herein differs from that disclosed in 55 said pending application in that the usual

annealing step is combined with the heat-treatment and such heat-treatment preferably takes place in an air or oxygen free atmosphere.

Galvanized wire which is to be used for fabricating purposes and more particularly that which is to be used in the manufacture of woven wire fencing must have a relatively heavy coating of spelter in order to be able 60 to withstand atmospheric corroding conditions, and before my invention was developed this was not possible except at a much increased cost of production.

The universal practice for testing the 70 relative value of spelter on galvanized wire is by the so-called Preece or copper sulfate test. There are other tests, however, which are used for quantitatively determining the amount of spelter on galvanized wire, such 75 as stripping the coating in caustic soda solution; in a suitable hydrochloric acid solution; in a solution of hydrochloric acid and antimony chloride, and in a lead acetate solution. The copper sulfate test, although 80 not strictly quantitative, is comparative when used under known conditions of temperature and strength, and being a quick test, and one which can be performed by any one after a little experience, has come to be the routine 85 testing medium for galvanized wire coatings.

At the present time there are only two (2) methods in use whereby these necessary heavy zinc (spelter) coatings may be obtained by the hot process of galvanizing. 90 The first method is to pass the wire very slowly as it emerges from the galvanizing bath, through finely divided charcoal. By such a process a smooth, thick coating may be obtained. This method is used for making telephone wire. It has serious draw- 95 backs, however, from an economic standpoint, because the wire must travel at a very slow speed, a very high grade zinc must be used, and, furthermore, the coated wire can- 100 not be subjected to the action of wire-fence fabricating machines without having considerable of the zinc coating crack or flake off the iron base. The second method is to cause the wire to travel at relatively slow 105 speeds, through a bath of molten spelter, the speed depending on the gauge of wire, the thickness of coating desired and the length of the molten spelter bath, and then wiping the wire by passing it between suitable 110 wipers. In other words, a wire will have a heavier galvanized coating, as measured by

the copper sulfate test, the longer it remains in the molten spelter. This latter process, too, has its economic drawbacks, because of the slow speeds required, the long spelter 5 pans necessary and consequently the lessening of the tonnage passing through a galvanizing unit in a given time.

In the accompanying drawing there is illustrated diagrammatically the usual or ordinary continuous galvanizing or coating apparatus, except the annealing furnace which is not placed as it is ordinarily, and includes the "acid" bath, "flux" bath, "coating" or galvanizing bath, and my "heat-treater" associated therewith, which in this instance is used as a combined "heat-treater and annealer." There is also illustrated a means whereby an air or oxygen free atmosphere may be maintained within 10 my "heat-treater and annealer," wherein both ends of the "heat-treater and annealer" are sealed; one end being submerged below the surface of the coating bath and the other being submerged below the surface 15 of water, oil or some other sealing means. Thus when my combined "heat-treater and annealer" is heated all the oxygen in the confined air is soon used up and both ends being sealed no more 20 air can enter so long as the heat is maintained.

My process consists preferably in treating wire as is usual in the ordinary continuous coating of wire, except that the initial 25 annealing step is omitted. This step being combined with the heat-treatment to be described, which follows the coating step, and preferably in an air or oxygen free atmosphere. I have discovered that if after the 30 wire leaves the coating bath it is subjected to a temperature of approximately 1250° F. I not only have a superior coated wire but said wire is also annealed. I realize that annealing per se is not new, but is new 35 in conjunction with my heat-treatment of the coated wire. I also realize that the annealing temperature will vary for different carbon contents or kinds of wire, or whether the annealing is to relieve the strain 40 of "bench hardening" that comes from the cold working of the wire, or whether from some other source. For example, if a "bench hardened" No. 12 gauge wire (American steel wire gauge) the carbon content 45 of which is approximately 0.12% is passed through molten spelter, the temperature of which is approximately 870° F., for approximately two seconds and then through a heat-treater, preferably a heated tube held 50 at approximately 1250° F. and preferably free of air or oxygen, for approximately ten seconds, and with or without wiping after leaving the heat-treatment, a wire is 55 coated which will stand approximately four 60 one minute immersions in copper sulfate;

whereas another wire traveling through the spelter at the same time and speed as the treated wire and wiped after leaving the spelter, and not passing through the heat-treatment, will stand, as a general rule, not 70 over one one minute immersion in copper sulfate. If the latter wire (which I call the control wire) is not passed through a wipe of some kind after it leaves the spelter, then, although I obtain a wire which will 75 stand more than one copper sulfate immersion test, it is very rough, an uncommercial, unsalable product, and cannot be successfully used in fence fabricating machines.

What I have described for No. 12 gauge 80 wire is also true for other gauges of wire, some of the larger gauges such as No. 9 standing oftentimes many more than four copper sulfate immersion tests. I do not, of course, limit myself to the speeds and temperatures above given because I have found that I may vary the speeds by controlling the temperatures; for example, if I want the wire to travel at a high speed, then I use higher temperatures, and vice versa, 85 as clearly described in my copending application, above referred to.

"Heat-treatment" as employed by me has reference to such treatment as will produce a physical or chemical change in the material 90 undergoing treatment. "Annealing" is also a heat-treatment and refers to the softening of hard wire, such as "bench hardened" wire. It is well known that when wire is drawn it becomes harder after each reduction, due to physical changes which take place within its structure. This hardness may be relieved and the wire made soft by heating the wire to a much lower temperature than would be the case if the hardness 100 was due to "carbon hardness." For example—in a 0.12% carbon wire it is well known that in order to anneal for "carbon hardness" it is necessary to heat the wire in the neighborhood of 1650° F., whereas 110 heating to around 1250° F. will be sufficient to relieve the hardness caused by the drawing of the wire and expressed by me as "bench hardness."

It is well known that hard wire is unsuitable for use in many kinds of wire fabricating machines. For this reason the wire must be annealed. Heretofore this step has taken place preceding the coating of the wire, but in my new process, I do this subsequent to the coating of the wire and in conjunction with my heat-treating. This, of course, eliminates one complete step in the continuous galvanizing process and effects considerable economies from a cost 125 standpoint.

When the wire leaves the coating bath and is not wiped or smoothed an uneven brittle coating is the result. I therefore subject the coated material to a suitable heat- 130

treatment such as I have previously described. The result of this heat-treatment is a smooth, even, pliable coating and due to the fact that the coating was not wiped 5 there is a heavier coating on the wire than is the case with ordinary processes. Furthermore, when galvanized coatings are subjected to high temperatures in the presence of air or oxygen the zinc of the spelter burns 10 to zinc oxide. For this reason I find it preferable to exclude air or oxygen from my heat-treater.

Wire galvanized by my process has an exceptionally smooth coating even without 15 the use of wipes. This gives me another advantage, in that I eliminate the production of "reachers" which, with the ordinary galvanizing practice are always produced and as such are valueless except as scrap. 20 Furthermore, it is not necessary for me to use excessively long spelter pans, as I have eliminated the necessity for long immersion of the wire in molten spelter:

By eliminating the initial annealing step 25 and coordinating the annealing and heat-treatment after coating, I avoid the necessity of using a special furnace for the initial annealing and thus effect considerable economies over the usual and long established process.

What I claim is:—

1. The process of treating metal coated materials having an iron base which consists in subjecting the material to a heat-treatment in an air or oxygen free atmosphere. 35

2. The process of treating metal coated materials having an iron base which consists in subjecting the material to a heat-treatment in an air or oxygen free atmosphere, and continuously moving the material 40 through the heat.

3. The process of treating un-annealed metal coated materials having an iron base 45 which consists in simultaneously subjecting

the material to a heat-treatment and annealing in an air or oxygen free atmosphere.

4. The process of treating un-annealed metal coated materials having an iron base which consists in simultaneously subjecting 50 the material to a heat-treatment and annealing in an air or oxygen free atmosphere, and continuously moving the material during such heating and annealing.

5. The process of treating un-annealed 55 metal coated materials having an iron base which consists in simultaneously subjecting the material to a heat-treatment and annealing.

6. The process of treating un-annealed 60 metal coated materials having an iron base which consists in simultaneously subjecting the material to a heat-treatment and annealing, and continuously moving the material during such heating and annealing. 65

7. The process of galvanizing wire, which consists in continuously moving the wire and during such movement subjecting the same, first—to a molten bath of spelter and upon leaving the bath subjecting the coated wire 70 to a heat-treatment in an air or oxygen free atmosphere.

8. The process of galvanizing un-annealed wire, which consists in continuously moving the wire and during such movement subjecting the same, first—to a molten bath of spelter and upon leaving the bath subjecting the coated wire to a simultaneous annealing and heat-treatment in an air or oxygen free atmosphere. 75 80

9. The process of galvanizing un-annealed wire, which consists in continuously moving the wire and during such movement subjecting the same, first, to a molten bath of spelter and upon leaving the bath subjecting the coated wire to a simultaneous annealing and heat-treatment. 85

In witness whereof I have hereunto affixed my hand this 25th day of February, 1922.

JOSEPH L. HERMAN.